



US007767040B2

(12) **United States Patent**  
**Kosaka et al.**

(10) **Patent No.:** **US 7,767,040 B2**  
(45) **Date of Patent:** **Aug. 3, 2010**

(54) **TITANIUM ALLOY AND AUTOMOTIVE EXHAUST SYSTEMS THEREOF**

(75) Inventors: **Yoji Kosaka**, Henderson, NV (US);  
**Stephen P. Fox**, Henderson, NV (US)

(73) Assignee: **Titanium Metals Corporation**, Dallas, TX (US)

(\*) Notice: Subject to any disclaimer, the term of this patent is extended or adjusted under 35 U.S.C. 154(b) by 0 days.

(21) Appl. No.: **12/315,773**

(22) Filed: **Dec. 5, 2008**

(65) **Prior Publication Data**

US 2009/0129968 A1 May 21, 2009

**Related U.S. Application Data**

(63) Continuation of application No. 10/460,233, filed on Jun. 13, 2003, now abandoned.

(60) Provisional application No. 60/390,145, filed on Jun. 21, 2002.

(51) **Int. Cl.**

**C22C 14/00** (2006.01)

(52) **U.S. Cl.** ..... **148/421**; 420/417; 420/418

(58) **Field of Classification Search** ..... 148/421; 420/417, 418

See application file for complete search history.

(56) **References Cited**

U.S. PATENT DOCUMENTS

5,885,375 A \* 3/1999 Takemura et al. .... 148/421  
6,531,091 B2 \* 3/2003 Miyamoto et al. .... 420/418

FOREIGN PATENT DOCUMENTS

JP 10017961 A \* 1/1998

OTHER PUBLICATIONS

"ASM Handbook vol. 2", ASM International, 1990, p. 594.\*

\* cited by examiner

*Primary Examiner*—Roy King

*Assistant Examiner*—Janelle Morillo

(74) *Attorney, Agent, or Firm*—Locke Lord Bissell & Liddell, LLP

(57) **ABSTRACT**

An oxidation resistant, high strength titanium alloy, particularly adapted for use in the manufacture of automotive exhaust system components and other applications requiring oxidation resistance and strength at elevated temperatures. The alloy comprises, in weight percent, iron less than 0.5, or 0.2 to less than 0.5%, oxygen 0.02 to less than 0.15%, silicon 0.15 to 0.6%, and balance titanium. Optional alloying elements are Al, Nb, V, Mo, Sn, Zr, Ni, Cr and Ta, with a total content of less than 1.5.

**30 Claims, 1 Drawing Sheet**

Effect of Silicon Content on Oxidation  
Resistance in Ti-Si Binary Alloys



Effect of Silicon Content on Oxidation  
Resistance in Ti-Si Binary Alloys



FIG. 1

## 1

## TITANIUM ALLOY AND AUTOMOTIVE EXHAUST SYSTEMS THEREOF

## CROSS-REFERENCE TO RELATED APPLICATION

The current application is a continuation of U.S. application Ser. No. 10/460,233 now abandoned which claims the benefit of priority under 35 U.S.C. §119(e) to U.S. Provisional Application No. 60/390,145 filed Jun. 21, 2002, the contents of which are herein incorporated by reference.

## DESCRIPTION OF THE INVENTION

## 1. Field of the Invention

The invention relates to an oxidation resistant, high strength titanium alloy which may in the form of a flat rolled or coiled strip product. The alloy is advantageously used for automotive exhaust system components, wherein elevated temperature strength and oxidation resistance is a required combination of properties.

## 2. Background of the Invention

It is known to use commercially pure (CP) titanium for automotive exhaust systems and mufflers for motorcycles. These exhaust systems made of CP titanium are lighter than those made from standard stainless steel. Weight reductions when using titanium to replace stainless steel may be as high as 44%, which is equivalent to approximately 20 lbs. of weight reduction for the system.

The use of CP titanium in exhaust systems to benefit from the weight reduction results in commercially pure titanium exhibiting excessive oxidation and softening during this high temperature service application. Consequently, the use of CP titanium sheet product has been limited to specific components of exhaust systems that are exposed to relatively low temperatures.

Consequently, there is a demand from both the automotive and exhaust system manufacturers for a titanium alloy sheet product that can be used at higher temperatures than CP titanium sheet product. The critical properties for this product are oxidation resistance and elevated temperature strength at temperatures up to 1600 F. In addition, since this sheet product requires a forming and fabricating operation to produce the various exhaust system components, cold formability and weldability are required close to these properties exhibited by CP titanium.

## SUMMARY OF THE INVENTION

In accordance with the invention, an oxidation resistant, high strength titanium alloy comprises, in weight %, less than 0.5 iron, 0.02 to less than 0.15 oxygen, 0.15 to 0.6 silicon and balance titanium and incidental impurities. Iron may be present within the range of 0.2 to less than 0.5%.

The alloy may include at least one element of Al, Nb, V, Mo, Sn, Zr, Ni, Cr and Ta in a total amount of less than 1.5%.

The alloy preferably has a minimum UTS of 7 ksi upon testing at a temperature of 1400 F, in combination with resistance to oxidation at 1400 F for 100 hours of less than 1% weight gain.

The alloy may be in the form of a flat rolled product or a coil strip product.

## 2

The alloy may be in the form of an automotive exhaust system component, which may be a muffler.

With respect to the alloy composition in accordance with the invention, silicon is the most important alloying element.

5 Silicon is known to be effective in titanium alloys to improve strength and creep resistance at elevated temperatures. Silicon is also effective to suppress grain growth during long time exposure at elevated temperatures. If the content of silicon is too low, the effect will not be sufficient in this regard. On the other hand, if the content is too great, formability of resulting sheet product of the alloy will be deteriorated.

Oxygen is an effective strengthening element in titanium alloys at ambient temperatures, but has little affect on the 15 oxidation and strength at elevated temperatures. In accordance with the invention, if the content of oxygen is too low, the cost of the titanium sheet of the alloy will increase, because scrap metal will not be suitable for use in the melting 20 of the alloy. On the other hand, if the content is too great, formability will be deteriorated.

Iron is a strengthening element in titanium at ambient temperatures, but has a slightly inverse affect on oxidation. If, however, the iron content exceeds the upper limits in accordance 25 with the invention, there will potentially be a segregation problem and ductility and formability will consequently be reduced. On the other hand, having iron at an extremely low level will result in excessive raw material costs.

The elements Al, Nb, V, Mo, Sn, Zr, Ni, Cr, Cu and Ta may 30 be present in the alloy in accordance with the invention to improve specific properties. A total content of these elements is less than 1.5%.

## BRIEF DESCRIPTION OF THE DRAWINGS

FIG. 1 is a graph showing the effect of silicon on oxidation resistance in Ti—Si binary alloys.

## DETAILED DESCRIPTION AND SPECIFIC EXAMPLES

## Example 1

40 45 Button arc melt ingots each weighing approximately 225 grams were made. The chemical composition of each button is given in Table 1. The buttons were forged and hot rolled to sheets with about 0.12" thickness. The sheets were then cold rolled to about 0.050" followed by annealing at 1400 F for 10 minutes. After flash pickle to clean the surface, coupons were 50 55 cut for oxidation tests and tensile tests at both ambient and elevated temperatures. The oxidation tests were performed at 1300 F/100 hours in air. The results of the tests are summarized in Table 2. The invention alloys, C and D, exhibited higher strength than commercially pure titanium (CP Ti) particularly at elevated temperatures. This is due to the silicide precipitates in these alloys. The 3% aluminum containing alloys, A, B, E and F, show good oxidation resistance and strength. However, their ductility is not as good as invention 60 alloys.

55 60 Microstructural observations of the oxidized samples indicated that the alloys that did not contain silicon exhibited substantial grain coarsening after being exposed at high temperatures for long periods of time. These coarse grains could 65 potentially cause brittleness. In contrast, the silicon-containing alloys maintained relatively finer grains due to the pinning effect of silicides and the beta phase.

TABLE 1

| Chemical Composition of Test Materials (wt %) |                  |      |      |      |     |      |            |
|-----------------------------------------------|------------------|------|------|------|-----|------|------------|
| Alloy                                         | Alloy Type       | Al   | Fe   | Si   | Nb  | O    | Remarks    |
| A                                             | Ti—0.5Si—3Al—1Nb | 3.0  | 0.07 | 0.42 | 1.0 | 0.12 | Comparison |
| B                                             | Ti—0.5Si—3Al     | 3.0  | 0.06 | 0.40 | —   | 0.12 | Comparison |
| C                                             | Ti—0.5Si—1Nb     | 0.01 | 0.06 | 0.44 | 1.0 | 0.12 | Invention  |
| D                                             | Ti—0.5Si         | 0.01 | 0.07 | 0.42 | —   | 0.12 | Invention  |
| E                                             | Ti—3Al—1Nb       | 2.9  | 0.22 | 0.01 | 0.9 | 0.11 | Comparison |
| F                                             | Ti—3Al           | 3.0  | 0.06 | 0.01 | —   | 0.11 | Comparison |
| G                                             | Ti—1Nb           | 0.02 | 0.08 | 0.01 | 1.0 | 0.11 | Comparison |
| H                                             | CP Ti            | 0.01 | 0.06 | 0.01 | —   | 0.10 | Comparison |
| Production Sheet Grade 2                      |                  | —    | 0.07 | 0.01 | —   | 0.14 | Comparison |
| Production Sheet Grade 12                     |                  | 0.01 | 0.13 | 0.02 | —   | 0.11 | Comparison |
| Ni: 0.89, Mo: 0.28                            |                  |      |      |      |     |      |            |

TABLE 2

| Results of Mechanical and Oxidation Tests |                  |             |             |           |                  |               |           |                |
|-------------------------------------------|------------------|-------------|-------------|-----------|------------------|---------------|-----------|----------------|
| Alloy                                     | Alloy Type       | UTS         | YS          | EI        | UTS              | Bend          | Oxidation |                |
|                                           |                  | (RT)<br>ksi | (RT)<br>ksi | (RT)<br>% | (800° F.)<br>ksi | Radius<br>(T) | WG<br>(%) | ASTM<br>GS No. |
| A                                         | Ti—0.5Si—3Al—1Nb | 86.8        | 80.2        | 19        | 52.0             | 6.5           | 0.29      | 9.0            |
| B                                         | Ti—0.5Si—3Al     | 88.6        | 80.8        | 23        | 50.6             | 2.2           | 0.35      | 7.5            |
| C                                         | Ti—0.5Si—1Nb     | 76.7        | 72.3        | 28        | 38.2             | 0.3           | 0.44      | 9.0            |
| D                                         | Ti—0.5Si         | 75.9        | 69.3        | 28        | 38.5             | 0.2           | 0.44      | 9.5            |
| E                                         | Ti—3Al—1Nb       | 76.5        | 67.7        | 27        | 38.3             | 2.0           | 0.63      | 5.0            |
| F                                         | Ti—3Al           | 75.7        | 67.1        | 24        | 38.6             | 2.1           | 0.45      | 5.5            |
| G                                         | Ti—1Nb           | 60.8        | 47.8        | 32        | 21.1             | 0.3           | 0.62      | 5.0            |
| H                                         | CP Ti            | 56.2        | 43.4        | 36        | 19.5             | 0.3           | 0.89      | 3.5            |
| Production Sheet Grade 2                  |                  | 75.3        | 54.2        | 27        | 28.9             | 0.8           | 0.83      | 3.5            |
| Production Sheet Grade 12                 |                  | 84.4        | 59.4        | 27        | 49.1             | 0.6           | 1.14      | 10.0           |

## Example 2

Additional button arc melted ingots each weighing approximately 225 grams were made. The chemical composition of each button is given in Table 3. The buttons were forged and hot rolled to sheets of about 0.12" thickness. Then the sheets were cold rolled to about 0.050" followed by annealing at 1400 F for 10 minutes. After a flash pickle to clean the surface, coupons were cut for oxidation testing and tensile testing at both ambient and elevated temperatures. Oxidation testing was performed at 1300 F/100 hours. Selected samples were subject to the additional oxidation

35 testing at 1500 F/100 hours, which is considered to be a severe condition in automotive exhaust system applications.

The test results are summarized in Table 4. These test results show that the strength at room temperature or elevated 40 temperature increased with increases in silicon content. Also weight gain after the exposure in air at 1300 F for 100 hours decreases with increases in silicon content. This is also shown in FIG. 1. Oxidation testing at a much higher temperature of 45 1500 F indicated that the alloys with silicon contents less than 0.15% (Alloy 0 or P) did not exhibit equivalent oxidation resistance to those with higher silicon alloys (Alloy M or N).

TABLE 3

| Chemical Composition of Test Materials (wt %) |                         |      |      |      |      |      |            |
|-----------------------------------------------|-------------------------|------|------|------|------|------|------------|
| Alloy                                         | Alloy Type              | Al   | Fe   | Si   | Sn   | O    | Remarks    |
| I                                             | Ti—0.1Si                | 0.02 | 0.11 | 0.10 | —    | 0.15 | Comparison |
| J                                             | Ti—0.25Si               | 0.02 | 0.13 | 0.23 | —    | 0.21 | Comparison |
| K                                             | Ti—1Si                  | 0.02 | 0.11 | 0.92 | —    | 0.17 | Comparison |
| L                                             | Ti—0.5Fe                | 0.02 | 0.59 | 0.01 | —    | 0.18 | Comparison |
| M                                             | Ti—0.5Si—0.25Fe-Low O   | —    | 0.24 | 0.42 | —    | 0.12 | Invention  |
| N                                             | Ti—0.5Si—0.25Fe-High O  | —    | 0.27 | 0.46 | —    | 0.20 | Comparison |
| O                                             | Ti—0.15Si—0.25Fe-Low O  | —    | 0.26 | 0.14 | —    | 0.13 | Comparison |
| P                                             | Ti—0.15Si—0.25Fe-High O | —    | 0.19 | 0.09 | —    | 0.23 | Comparison |
| Q                                             | Ti—0.5Si—1Sn            | —    | 0.03 | 0.46 | 0.96 | 0.11 | Invention  |
| R                                             | Ti—1Sn                  | —    | 0.03 | 0.01 | 0.97 | 0.14 | Comparison |

The oxidation test also indicated that a sole addition of iron or tin without silicon did not show any benefit in terms of oxidation resistance (Alloy L or R). However, the addition of iron or tin with the addition of silicon showed equivalent oxidation resistance (Alloy M, N, O, P and Q). The effect of oxygen was mixed regarding strength. The strength at room temperature increases with oxygen (compare alloy M and N or O and P), but there was no affect on the strength or oxidation resistance at elevated temperatures.

The results of oxidation tests are given in Table 6. It is evident from the results that the invented alloys exhibited oxidation resistance superior to CP titanium at all temperatures. The difference in the oxidation resistance between the invented alloy sheets and CP titanium sheet increases with temperature. Table 7 shows the results of the tensile tests. These tests demonstrate that the invented alloy sheets exhibited higher strength than CP titanium sheet at all temperatures.

TABLE 4

| Results of Mechanical and Oxidation Tests |                         |      |      |      |           |                 |      |            |
|-------------------------------------------|-------------------------|------|------|------|-----------|-----------------|------|------------|
| Alloy                                     | Alloy Type              | UTS  | YS   | EI   | UTS       | Weight Gain (%) |      |            |
|                                           |                         | (RT) | (RT) | (RT) | (800° F.) |                 |      |            |
| I                                         | Ti—0.1Si                | 78.1 | 64.3 | 28   | 29.1      | 0.51            | n/a  | Comparison |
| J                                         | Ti—0.25Si               | 82.0 | 70.3 | 34   | 34.4      | 0.51            | n/a  | Comparison |
| K                                         | Ti—1Si                  | 94.3 | 82.8 | 24   | 46.6      | 0.36            | n/a  | Comparison |
| L                                         | Ti—0.5Fe                | 87.9 | 71.5 | 27   | 34.2      | 0.83            | n/a  | Comparison |
| M                                         | Ti—0.5Si—0.25Fe-Low O   | 80.3 | 72.7 | 25   | 42.3      | 0.40            | 1.56 | Invention  |
| N                                         | Ti—0.5Si—0.25Fe-High O  | 89.8 | 80.1 | 27   | 40.9      | 0.41            | 1.59 | Comparison |
| O                                         | Ti—0.15Si—0.25Fe-Low O  | 72.0 | 61.6 | 22   | 32.9      | 0.52            | 2.59 | Comparison |
| P                                         | Ti—0.15Si—0.25Fe-High O | 86.0 | 74.7 | 20   | 31.7      | 0.49            | 2.25 | Comparison |
| Q                                         | Ti—0.5Si—1Sn            | 75.6 | 67.3 | 25   | 36.5      | 0.28            | 2.78 | Invention  |
| R                                         | Ti—1Sn                  | 63.2 | 48.7 | 28   | 20.5      | 0.81            | 13.9 | Comparison |

(Duration of oxidation test is 100 hours at given temperatures)

## Example 3

Two alloy ingots each of about 18 lbs. were made with a laboratory VAR (Vacuum Arc Remelting) furnace. The ingots were made with a double VAR process, which is frequently used in the production of titanium ingots. The ingots were forged to 1.0" thick plates, followed by hot rolling to 0.125" thick plates. After blast and pickle to remove scale and alpha case, the plates were cold rolled to 0.050" thick sheets followed by annealing at 1400 F/10 min. and flash pickle. The sheets were produced without any hot or cold rolling problems. Table 5 shows the chemical composition of these alloys. Various tests were performed on the sheets to verify the superiority in properties required for automotive exhaust materials compared to CP titanium Grade 2.

40 Welding is employed in the production of exhaust tubes and other components, and in the assemble of exhaust systems. Both autogenous welding and welding with filler metal are used. Table 8 shows the results of tensile testing after 45 welding with gas tungsten arc welding (GTAW). A CP titanium wire was used for filler metal. Although the microstructure of the weldment and part of heat affected zone exhibited a transformed beta microstructure with coarse grains, the welds had sufficiently high strength with an acceptable ductility.

TABLE 5

| Chemical Composition of Test Materials (wt %) |                |      |      |      |      |       |            |
|-----------------------------------------------|----------------|------|------|------|------|-------|------------|
| Alloy                                         | Alloy Type     | Si   | Fe   | C    | O    | N     | Remarks    |
| S                                             | Ti—0.5Si       | 0.54 | 0.13 | 0.06 | 0.11 | 0.001 | Invention  |
| T                                             | Ti—0.5Si—0.5Fe | 0.42 | 0.49 | 0.05 | 0.10 | 0.002 | Invention  |
| Prod. Sheet Grade 2                           |                | 0.01 | 0.07 | 0.01 | 0.14 | 0.008 | Comparison |

TABLE 6

| <u>Results of Oxidation Test</u> |                |         |         |         |         |            |
|----------------------------------|----------------|---------|---------|---------|---------|------------|
| Alloy                            | Alloy Type     | 1300 F. | 1400 F. | 1500 F. | 1600 F. | Remarks    |
| S                                | Ti—0.5Si       | 0.58    | 0.70    | 1.66    | 3.18    | Invention  |
| T                                | Ti—0.5Si—0.5Fe | 0.49    | 0.73    | 1.93    | 4.25    | Invention  |
| Prod. Sheet Grade 2              |                | 1.03    | 3.01    | 20.02   | 37.14   | Comparison |

(weight gain % after exposure in air for 100 hours at given temperature)

TABLE 7

| <u>Results of Tensile Tests at Room Temperature and Elevated Temperatures</u> |                |      |      |        |      |         |     |
|-------------------------------------------------------------------------------|----------------|------|------|--------|------|---------|-----|
| Alloy                                                                         | Alloy Type     | RT   |      | 800 F. |      | 1400 F. |     |
|                                                                               |                | UTS  | YS   | UTS    | YS   | UTS     | YS  |
| S                                                                             | Ti—0.5Si       | 81.7 | 74.8 | 42.6   | 37.1 | 9.1     | 8.9 |
| T                                                                             | Ti—0.5Si—0.5Fe | 84.3 | 76.1 | 45.4   | 37.9 | 9.2     | 9.0 |
| Prod. Sheet Grade 2                                                           |                | 68.2 | 55.9 | 25.9   | 22.2 | 5.7     | 5.7 |

TABLE 8

| <u>RT Tensile Properties of Welded Sheets</u> |                |                   |      |                      |      |      |
|-----------------------------------------------|----------------|-------------------|------|----------------------|------|------|
| Alloy                                         | Alloy Type     | With Filler Metal |      | Without Filler Metal |      |      |
|                                               |                | UTS               | YS   | EI                   | UTS  | YS   |
| S                                             | Ti—0.5Si       | 89.9              | 69.9 | 9                    | 92.8 | 78.0 |
| T                                             | Ti—0.5Si—0.5Fe | 96.9              | 83.8 | 7                    | 98.6 | 82.0 |

Other embodiments of the invention will be apparent to those skilled in the art from consideration of the specification and practice of the invention disclosed herein. It is intended that the specification and examples be considered as exemplary only, with a true scope and spirit of the invention being indicated by the following claims.

All percentages are in percent by weight in both the specification and claims.

What is claimed is:

1. An oxidation resistant, high strength titanium alloy consisting essentially of, in weight %, 0.2 to less than 0.5 iron, 0.02 to less than 0.12 oxygen, 0.15 to 0.42 silicon and balance titanium and incidental impurities.

2. The alloy of claim 1, additionally consisting essentially of at least one element selected from the group consisting of Al, Nb, V, Mo, Sn, Zr, Ni, Cr and Ta, with a total content of less than 1.5.

3. The alloy of claim 2 having a minimum UTS of 7 ksi upon testing at a temperature of 1400 F in combination with resistance to oxidation at 1400 F for 100 hours of less than 1% weight gain.

4. A flat rolled product of an oxidation resistant, high strength titanium alloy consisting essentially of, in weight %, 0.2 to less than 0.5 iron, 0.02 to less than 0.12 oxygen, 0.15 to 0.42 silicon and balance titanium and incidental impurities.

5. The flat rolled product of claim 4 wherein said alloy additionally consists essentially of at least one element selected from the group consisting of Al, Nb, V, Mo, Sn, Zr, Ni, Cr and Ta, with a total content of less than 1.5.

6. The flat rolled product of claim 4 in the form of a plate.

7. The flat rolled product of claim 4 in the form of a sheet.

35 8. Coil strip products, produced by combinations of hot strip rolling, cold strip rolling and annealing, of an oxidation resistant, high strength titanium alloy consisting essentially of, in weight %, 0.2 to less than 0.5 iron, 0.02 to less than 0.12 oxygen, 0.15 to 0.42 silicon and balance titanium and incidental impurities, said alloy having a minimum UTS of 7 ksi upon testing at a temperature of 1400 F in combination with resistance to oxidation at 1400 F for 100 hours of less than 1% weight gain.

40 9. The coiled product of claim 8 wherein said alloy additionally consists essentially of at least one element selected from the group consisting of Al, Nb, V, Mo, Sn, Zr, Ni, Cr and Ta, with a total content of less than 1.5.

45 10. An automotive exhaust system component comprising an oxidation resistant, high strength titanium alloy consisting essentially of, in weight %, 0.2 to less than 0.5 iron, 0.02 to less than 0.12 oxygen, 0.15 to 0.42 silicon and balance titanium and incidental impurities.

50 11. An automotive exhaust system component of claim 10 wherein said alloy additionally consists essentially of at least one element selected from the group consisting of Al, Nb, V, Mo, Sn, Zr, Ni, Cr and Ta, with a total content of less than 1.5.

55 12. An automotive exhaust system component of claim 11 wherein said alloy has a minimum UTS of 7 ksi upon testing at a temperature of 1400 F in combination with resistance to oxidation at 1400 F for 100 hours of less than 1% weight gain.

60 13. A muffler comprising an oxidation resistant, high strength titanium alloy consisting essentially of, in weight %, 0.2 to less than 0.5 iron, 0.02 to less than 0.12 oxygen, 0.15 to 0.42 silicon and balance titanium and incidental impurities.

**14.** A muffler comprising an oxidation resistant, high strength titanium alloy of claim 13 wherein said alloy additionally consists essentially of at least one element selected from the group consisting of Al, Nb, V, Mo, Sn, Zr, Ni, Cr and Ta, with a total content of less than 1.5.

**15.** A muffler comprising an oxidation resistant, high strength titanium alloy of claim 14 wherein said alloy has a minimum UTS of 7 ksi upon testing at a temperature of 1400 F in combination with resistance to oxidation at 1400 F for 100 hours of less than 1% weight gain.

**16.** A flat rolled product comprising a plate of a titanium alloy consisting essentially of, in weight %, 0.2 to less than 0.5 iron, 0.02 to less than 0.12 oxygen, 0.15 to 0.42 silicon and balance titanium and incidental impurities.

**17.** The flat rolled product of claim 16 wherein said titanium alloy additionally consists essentially of at least one element selected from the group consisting of Al, Nb, V, Mo, Sn, Zr, Ni, Cr and Ta, with a total content of less than 1.5.

**18.** The flat rolled product of claim 16 wherein said titanium alloy has a minimum UTS of 7 ksi upon testing at a temperature of 1400° F. in combination with a resistance to oxidation at 1400° F. for 100 hours of less than 1% weight gain.

**19.** A flat rolled product comprising a sheet of a titanium alloy consisting essentially of, in weight %, 0.2 to less than 0.5 iron, 0.02 to less than 0.12 oxygen, 0.15 to 0.42 silicon and balance titanium and incidental impurities.

**20.** The flat rolled product of claim 19 wherein said titanium alloy additionally consists essentially of at least one element selected from the group consisting of Al, Nb, V, Mo, Sn, Zr, Ni, Cr and Ta, with a total content of less than 1.5.

**21.** The flat rolled product of claim 19 wherein said titanium alloy has a minimum UTS of 7 ksi upon testing at a temperature of 1400° F. in combination with a resistance to oxidation at 1400° F. for 100 hours of less than 1% weight gain.

**22.** A flat rolled product comprising a coil strip of a titanium alloy consisting essentially of, in weight %, 0.2 to less than 0.5 iron, 0.02 to less than 0.12 oxygen, 0.15 to 0.42 silicon and balance titanium and incidental impurities.

**23.** The flat rolled product of claim 22 wherein said titanium alloy additionally consists essentially of at least one element selected from the group consisting of Al, Nb, V, Mo, Sn, Zr, Ni, Cr and Ta, with a total content of less than 1.5.

**24.** The flat rolled product of claim 22 wherein said titanium alloy has a minimum UTS of 7 ksi upon testing at a temperature of 1400° F. in combination with a resistance to oxidation at 1400° F. for 100 hours of less than 1% weight gain.

**25.** An elevated-temperature oxidation resistant, high strength titanium alloy consisting essentially of, in weight %, 0.2 to less than 0.5 iron, 0.02 to less than 0.12 oxygen, 0.15 to 0.42 silicon and balance titanium and incidental impurities.

**26.** The alloy of claim 25 wherein said titanium alloy additionally consists essentially of at least one element selected from the group consisting of Al, Nb, V, Mo, Sn, Zr, Ni, Cr and Ta, with a total content of less than 1.5.

**27.** The alloy of claim 25 wherein said alloy has a minimum UTS of 7 ksi upon testing at a temperature of 1400° F. in combination with a resistance to oxidation at 1400° F. for 100 hours of less than 1% weight gain.

**28.** An alloy having a minimum UTS of 9 ksi upon testing at a temperature of 1400 F in combination with resistance to oxidation at 1400 F for 100 hours of less than 0.8% weight gain consisting essentially of, in weight %, 0.2 to less than 0.5 iron, 0.02 to less than 0.12 oxygen, 0.15 to 0.42 silicon and balance titanium and incidental impurities.

**29.** A titanium alloy consisting essentially of, in weight %, 0.49 iron, 0.10 oxygen, 0.42 silicon and balance titanium and incidental impurities, said alloy having a minimum UTS of 9 ksi upon testing at a temperature of 1400 F in combination with resistance to oxidation at 1400 F for 100 hours of less than 0.8% weight gain.

**30.** An automotive exhaust system component comprising a titanium alloy consisting essentially of, in weight % 0.2 to less than 0.5 iron, 0.02 to less than 0.12 oxygen, 0.15 to 0.42 silicon and balance titanium and incidental impurities, said alloy having a minimum UTS of 7 ksi upon testing at a temperature of 1400 F in combination with resistance to oxidation at 1400 F for 100 hours of less than 1% weight gain.

\* \* \* \* \*